

Feb. 27, 1934.

K. A. LINDNER

1,949,392

## PROCESS FOR REACTING GASES WITH LIQUIDS

Original Filed Aug. 22, 1930



INVENTOR  
*Karl A. Lindner*  
BY  
*Austin & Dix*  
ATTORNEYS

## UNITED STATES PATENT OFFICE

1,949,392

## PROCESS FOR REACTING GASES WITH LIQUIDS

Karl A. Lindner, Roselle Park, N. J., assignor to  
American Smelting and Refining Company,  
New York, N. Y., a corporation of New Jersey

Original application August 22, 1930, Serial No.  
476,971. Divided and this application July 30,  
1932. Serial No. 626,601

8 Claims. (Cl. 75—15)

This invention relates to metal refining and more particularly to a process for reacting a gaseous reagent with a liquid, such as a molten metal. The present application is a division of my co-pending application, Serial No. 476,971, filed August 22, 1930.

The invention provides an improved method whereby a gaseous reagent may be reacted with a molten metal to eliminate impurities from the latter. For example, the invention is particularly suited for the removal of impurities, such as zinc, from a molten bath of lead by means of chlorine gas. For this purpose, a cylindrical reaction chamber is provided into which the gaseous chlorine is introduced. A stream of lead is pumped out of the bath of molten metal and is applied to the reaction chamber tangentially whereby it is caused to whirl therein and to come into intimate contact with the chlorine.

20 The reaction chamber is also provided with a conical base which extends almost to the level of the molten metal. This permits the slag to be washed out of the chamber by means of the molten metal and prevents the apparatus from 25 becoming clogged. Furthermore, the construction permits the apparatus to be started when the lead is at a temperature just above the melting point thereof, inasmuch as danger of lead freezing in the chamber and interrupting the 30 operation of the apparatus is avoided.

Although the novel features which are believed to be characteristic of this invention will be particularly pointed out in the claims appended hereto, the invention itself, as to its objects and 35 advantages, the mode of its operation and the manner of its organization may be better understood by referring to the following description taken in connection with the accompanying drawing forming a part thereof, in which

40 Fig. 1 is a plan view of a kettle showing the refining apparatus applied thereto; and

Fig. 2 is a side elevation of the apparatus showing the kettle in section and illustrating the relative position of the different elements.

45 Like reference characters denote like parts in the several figures of the drawing.

In the following description and in the claims 50 parts will be identified by specific names for convenience, but they are intended to be as generic in their application to similar parts as the art will permit.

55 Referring to the drawing more in detail, the invention is shown as applied to a kettle 10 which is supported by a rim 11 from any suitable frame-

work 12 and may be heated in any manner well known in the art.

The refining apparatus comprises a cylindrical reaction chamber 15 which is supported on a pair of beams 16 extending across the kettle and resting on the rim thereof. Said chamber 15 is provided with a gas inlet pipe by means of which the gaseous reagent may be applied thereto and has a conical bottom 19 terminating in a discharge pipe 20 which extends below the surface of the 60 bath 21 whereby the molten metal may completely react with the gaseous reagent and escape of said reagent from the top of the bath is avoided.

The reaction chamber is also provided with a tangential inlet pipe 22 by means of which the 70 molten metal is pumped into the chamber and caused to whirl around therein and to be broken up into small particles whereby an increased surface contact between the metal and the gaseous reagent is obtained. For removing a stream of metal from the bath and applying the same to inlet pipe 22 a pump 24 is provided, preferably of the centrifugal type, having an intake 25 and a discharge pipe 26 which extends from said pump into engagement with pipe 22. Pump 24 is driven 80 by motor 27 through a reducing gear 28 and a driving shaft 29 which are all mounted on beams 16. Said driving shaft serves to support the pump whereby the entire mechanism including the reaction chamber 15, pump 24, motor 27 and 85 gear 28 may be removed from the kettle as a unit.

In the operation of the above described apparatus in connection with the dezincing of lead, the pump may be started when the lead has been 90 heated to a comparatively low temperature, as for example, 635° F. Since the discharge pipe 20 is immersed in the molten lead and the level of the molten lead practically reaches the conical base 19, there is but little tendency for the metal within the chamber to freeze when the apparatus is started, even though it is applied to the bath at a temperature not greatly above the melting point thereof.

In reacting lead with chlorine a considerable 100 amount of heat is evolved and the temperature of the bath gradually increases. It is accordingly an advantage to start the apparatus at as low a temperature as possible in order to complete the dezincing operation before the bath has reached an excessively high temperature. The operation should preferably be discontinued when the lead reaches a temperature of approximately 775° F. inasmuch as above this temperature the tendency of the lead to react with the chlorine is in- 105 110

creased and the zinc chloride slag tends to be volatilized.

The tangential feed of the lead breaks up the flow of the metal and allows an intimate contact to be made with the chlorine. Furthermore, the tangential flow on the side of the chamber removes all slag particles and maintains the chamber free therefrom. It is obvious that the centrifugal force resulting from the pumping of the metal in a tangential direction against the curvilinear surface of the chamber combined with the force of gravity will cause the metal to follow a substantially spiral path against the walls of the chamber and to spread out and form a substantially continuous surface thereover. A continuously changing cylinder of metal is thus provided which serves as a lining for the chamber and shields the walls from contact with the reagent. The gaseous reagent within the cylinder contacts with the exposed surface of this metal lining and the products of the reaction, which are lighter than the metal itself, are separated therefrom by the centrifugal action of the moving metal and are caused to segregate toward the center of the chamber, thereby forming essentially an inner cylindrical coating which is drawn downwardly as a continuous core at the bottom of the chamber. This core is withdrawn as such through discharge pipe 20 into the sub-adjacent bath of metal and is permitted to float to the surface of said bath. Due to the fact that slag or reaction products are initially separated and agglomerated in the reaction chamber there is substantially no dispersion of slag particles through the bath of treated metal and a substantially complete separation of the two products is thereby facilitated.

It will be noted that the moving lining of molten metal and slag forms a protective coating over the inner surface of the chamber and thereby prevents the reactive gas from coming into contact with the metal walls and reduces the amount of corrosion which would otherwise take place due to the corrosive properties of the reactive gas. This materially increases the life of the reaction chamber and decreases the maintenance cost. Furthermore, the products of the reaction are swept out of the chamber, together with the unreacted metal and are prevented from accumulating at the bottom of the chamber and clogging the same or otherwise interfering with the operation of the apparatus.

By pumping the lead at the side and exposing a large surface to the chlorine it is possible to admit the chlorine at a comparatively rapid rate. For example, in a particular installation using a 100 ton kettle the chlorine was admitted at an average rate of 510 lbs. per hour. During the first two hours when the charge is saturated with zinc a larger quantity is admitted, for example, 600 lbs. per hour, but as the zinc becomes depleted the rate of feed of chlorine is reduced to prevent it from escaping through the outlet pipe 20. When the zinc has been depleted to .02% less zinc chloride begins to form and indicates to the operator that the charge has been completely dezincined. At this point the chlorine is shut off and the lead flow continued until all slag has been washed from the chamber.

The above apparatus has been particularly described as applied to the dezincining of lead by the introduction of chlorine and the formation of zinc chloride. However, it is not to be limited to this use, but is suitable for the reaction of

various gases with a liquid. The above use has been described by way of illustration only.

While certain novel features of the invention have been shown and described and are pointed out in the annexed claims, it will be understood that various omissions, substitutions and changes in the forms and details of the device illustrated and in its operation may be made by those skilled in the art without departing from the spirit of the invention.

What is claimed is:

1. The process of applying a gaseous reagent to a liquid in a reaction chamber which comprises tangentially introducing the liquid into said chamber thereby causing the liquid to spread out over the walls of said chamber and form a substantially continuous lining thereover whereby the walls of the chamber are shielded from contact with the gaseous reagent and a large surface area of said liquid is presented to said reagent, introducing the gaseous reagent into said chamber in controlled quantities whereby an appreciable excess of said reagent is avoided, and continuously withdrawing the liquid together with the products of reaction from said chamber. 100

2. The process of applying a gaseous reagent to a liquid in a reaction chamber which comprises introducing the liquid into said chamber in a tangential direction and causing said liquid to follow a substantially spiral path around the 105 walls of said chamber and to spread out over the surface thereof whereby said surface is shielded from contact with the gaseous reagent, introducing said reagent into said chamber in quantities calculated to react with said liquid 110 and utilizing the centrifugal force of said liquid to separate the products of reaction and cause the same to form a core at the bottom of said chamber and removing said core together with the unreacted liquid. 115

3. The process of treating molten lead with chlorine in a reaction chamber which comprises tangentially introducing the molten lead to said chamber thereby causing said lead to spread out over the inner surface of said chamber and shield 120 the surface from contact with chlorine, introducing chlorine to said chamber in quantities calculated to react with the impurities in said lead whereby an excess of chlorine is avoided, and continuously withdrawing the products of reaction 125 from said chamber together with the unreacted molten metal.

4. The process of treating molten lead with chlorine in a reaction chamber which comprises applying the molten lead to said chamber and 130 causing the same to spread out over the surface thereof, and to shield the surface from contact with chlorine, introducing chlorine to said chamber in quantities calculated to react with the impurities in said lead whereby an excess of chlorine 135 is avoided, and utilizing the centrifugal force due to movement of the lead over the walls of said chamber for separating the products of reaction and maintaining said products out of contact with the walls of said chamber and continuously withdrawing said products from said chamber together with the unreacted molten metal. 140

5. The process of reacting a liquid metal with a gaseous reagent which comprises causing said liquid to form a continuously moving, substantially hollow body, reacting the inner surface of the so-formed hollow body with said gaseous reagent, and continuously removing the unreacted liquid and the products of reaction from the lower extremity of said hollow body. 145

6. The process of reacting molten lead with a chlorine gas reagent in a substantially cylindrical chamber which comprises causing said lead to form a continuously moving, substantially hollow body, reacting the inner surface of the so-formed hollow body with said reagent, and continuously removing the unreacted lead and the products of reaction from the chamber.

7. The process of reacting a liquid with a gaseous reagent which comprises causing said liquid to form a continuously moving, substantially hollow body, reacting the inner surface of the so-formed hollow body with said gaseous reagent,

and continuously removing the unreacted liquid and the products of reaction as separate unmixed materials.

8. In refining lead contaminated with zinc, the method which consists of introducing a molten stream of such lead into a cylindrical reaction chamber at a tangent thereby causing the molten lead to substantially cover the walls of said reaction chamber, introducing chlorine gas into said chamber and withdrawing the reaction products from said chamber.

KARL A. LINDNER.

15

80

20

85

25

90

30

95

35

100

40

105

45

110

50

115

120

125

135

140

145

150